

## UNITED STATES PATENT OFFICE

2,148,033

## CARROTING PROCESS

Warren C. Mercier, Danbury, Conn., assignor to  
 American Hatters and Furriers Company, Incorporated, Danbury, Conn., a corporation of New York

No Drawing. Original application December 11, 1937, Serial No. 179,267. Divided and this application August 10, 1938, Serial No. 234,138

2 Claims. (Cl. 8—112)

This invention relates to a carroting process, an art of imparting proper felting characteristics to fur fibers.

This application is a division of my copending application Serial No. 179,267, filed December 11, 1937, which application is a continuation in part of applications Serial No. 532,699, filed April 24, 1931 and Serial No. 104,707, filed October 8, 1936.

10 One of the objects of this invention is to provide a carroting process which will be instrumental in providing fur fibers having one or more of the following characteristics:—mutual affinity resulting in a strong tight felt; an ability to felt with large quantities of non-feltable material known as filler; fast shrinking and quick starting during the felting operation; an absence of discoloration; no deterioration, in fact, improvement during substantial periods of storage; an ability to take all dye shades without objectionable "undercasts" or other mottled effects; a satisfactory weight for economical use in hat manufacture. Another object of this invention is to provide a carroting process utilizing a non-mercury carrot with a resulting economy and other advantages in hat manufacture. Other objects will be in part obvious and in part pointed out hereinafter.

The invention contemplates the utilization of novel combinations of chemical reagents for the treatment of furs as will be illustratively described herein, and the scope of the invention will be indicated in the following claims.

Briefly, felt, for example, the felt used in hat manufacture, comprises a compact mass of interlocking or interfitting fur fibers. In hat manufacture the fibers are deposited on a large cone in matted down condition and by a wetting and hardening process they are made to cling together in mutual adherence to form a hat body much too large in size and of flimsy texture. Such bodies are carefully removed from the cone and subjected to a series of operations which reduce the hat to its normal size and at the same time cause a tight interlocking of the individual fibers to provide a strong felt. Such operations may be briefly described as shrinking, rubbing and pounding under a variety of conditions with many types of machines and naturally the greater the speed of such operations the greater the resultant economy in hat manufacture. Two of the most important operations are known as "starting" and "sizing" in the hatting industry. Fur fibers which are quick to start and fast in sizing are obviously desirable in hat manufacture.

Fur fibers in their natural state are unsuitable for the felting operation and must be processed prior thereto; this process is generally known in the art as carroting. Regardless of

the quality of fur fibers, they are not suited for the felting operation unless the carroting process is carried out effectively prior thereto. This carroting process is usually accomplished by 5 combing a chemical solution into the fur fibers before they are removed from the pelt. After this, the fur is dried and subsequently cut from the pelts when it is ready for the felting operation. In practice, however, carroted fur is generally stored for substantial periods of time and 10 the process must be such that the fur will not deteriorate during this storage period.

Although several factors should be continually borne in mind to complete the carroting process in a successful manner, most important is the composition of the carroting solution. Such solutions should be free from toxic 15 effects to protect laborers coming into contact therewith during the felting operation. Obviously the carroting solution should be inexpensive to reduce the ultimate cost of felt manufacture. As noted above, fur is often stored for substantial periods of time; therefore, the carroting composition should be free from any ingredients injurious to the fibers during such 20 periods of storage. Felt is usually dyed, especially in the hatting industry and accordingly the carroted fur should be able to take all shades of dyes without undesirable "undercasting" or 25 mottled effects. So that the felting operation 30 may be rapid, fur fibers should have quick starting and fast sizing characteristics.

"Mercury carrot" comprising mercury nitrate in an excess of nitric acid has been the accepted carroting composition in the hatting industry for 35 many years because of several desirable characteristics. Fur carroted with this mercury carrot may be stored for substantial periods of time for it improves with age and the mercury carrot adds a considerable amount of weight 40 to the fibers. Fur carroted with the mercury carrot will also take a considerable amount of filler without affecting the quality of the resulting felt. In spite of these advantages, fur carroted with the mercury carrot has a definite 45 toxic effect which often seriously impairs the health of laborers coming in contact with the fur and it discolors the fur making it impossible to use light pastel dye shades on the resultant felt, thus often creating mottled effects even when 50 the dark dyes are used.

Because the mercury carrot has these disadvantages several non-mercury carrots have been developed with limited success. Although such non-mercury carrots have proven practical in 55 certain limited fields, they are all subject to one deficiency or another, making them unsuitable for universal use. Sometimes the fur does not take on enough weight when such carrots are used. With other non-mercury carrots the fur 60

deteriorates during storage. Still other non-  
mercury carrots have slow starting and sizing  
characteristics. For these and other reasons the  
mercury carrot is still preponderantly used in  
hat manufacture in spite of the above-noted  
disadvantages thereof.

The principal object of this invention has  
been to provide an inexpensive and practical non-  
mercury carrot free from the disadvantages there-  
of noted above.

It is now generally recognized that a carrott-  
ing solution should include a hydrolyzing agent  
and an oxidizing agent. The particular reasons  
why such ingredients are necessary constituents  
in a carrott-ing solution is not definitely known  
but successful carrott-ing solutions now in use in-  
clude such ingredients in one form or another.  
A carrott-ing solution comprising chloric acid and  
sulphuric acid has been suggested but after ex-  
tensive research this carrot has proven a failure.  
One of the principal objections to this carrott-ing  
solution is its slow starting and slow sizing char-  
acteristics, a disadvantage practically eliminating  
it for use in commercial operations. I have dis-  
covered that by the addition of certain peroxygen  
compounds to a solution of chloric and sulphuric  
acids, the above deficiencies thereof are success-  
fully remedied and the result is an excellent car-  
rot well adapted for commercial use.

30 My preferred carrott-ing solution comprises a  
solution of chloric acid, sulphuric acid and am-  
monium persulphate. It is my belief that the  
chloric acid and the ammonium persulphate are  
the primary oxidizing agents and the sulphuric  
35 acid is a hydrolyzing agent. Under certain cir-  
cumstances, I have obtained favorable results by  
substituting nitric acid for the sulphuric acid in  
this carrot so that the carrot comprises chloric  
acid, nitric acid and ammonium persulphate.  
40 Also, under certain conditions, I may substitute  
for the ammonium persulphate in this carrott-ing  
solution hydrogen peroxide, potassium permanganate,  
ammonium perchlorate, and sodium per-  
chlorate. Thus, the solution or solutions used  
45 include a strong hydrolyzing agent and a pro-  
nounced oxidizing agent. Preferably I employ  
two hydrolyzing agents, one at least of which is  
a strong hydrolyzing agent and a strong oxidizing  
agent. Preferably in one embodiment one of the  
50 hydrolyzing agents is chloric acid, and if a second  
hydrolyzing agent is used I prefer to use sul-  
phuric acid; the oxidizing agent may be hydrogen  
peroxide.

Accordingly, in summation, this carrott-ing solu-  
55 tion comprises chloric acid, nitric acid or sul-  
phuric acid, and any one of ammonium per-  
sulphate, sodium perchlorate, ammonium per-  
chlorate, hydrogen peroxide, or potassium per-  
manganate. When hydrogen peroxide is used in  
60 this solution, the strength thereof should be  
somewhere between 25 and 50 volumes.

Due to many factors to be taken into considera-  
tion when testing carrott-ing solutions, I am unable  
65 at the present time to give exact values and pro-  
portions of the various ingredients comprising  
the above carrott-ing solutions. However, my re-  
search has succeeded to such an extent that I  
have obtained satisfactory results with the solu-  
tions to follow, it being understood that these  
70 are merely illustrative examples and may vary  
widely in accordance with particular condi-  
tions:—

#### Example 1

|                        | Molal |
|------------------------|-------|
| Chloric acid           | .4    |
| Sulphuric acid         | .3    |
| Potassium permanganate | .15   |

#### Example 2

|                    | Molal |
|--------------------|-------|
| Chloric acid       | .35   |
| Sulphuric acid     | .3    |
| Sodium perchlorate | .8    |

#### Example 3

|                      | Molal |
|----------------------|-------|
| Chloric acid         | .25   |
| Sulphuric acid       | .2    |
| Ammonium perchlorate | .85   |

#### Example 4

|                   | Molal              |
|-------------------|--------------------|
| Chloric acid      | .55                |
| Sulphuric acid    | .8                 |
| Hydrogen peroxide | volume strength 50 |

#### Example 5

|                      | Molal |
|----------------------|-------|
| Chloric acid         | .55   |
| Sulphuric acid       | .8    |
| Ammonium persulphate | .8    |

#### Example 6

|                      | Molal |
|----------------------|-------|
| Nitric acid          | .4    |
| Chloric acid         | .6    |
| Ammonium persulphate | .7    |

These solutions are generally combed into the  
fur while it is still on the pelts and, after dry-  
ing, the fur is cut from the pelts and used in the  
felting operation or stored. Fur so carrott-ed may  
be used with absolute safety during the felting  
process without any toxic effects and the in-  
gredients comprising the above solutions are rela-  
tively inexpensive, thus materially reducing the  
cost of the carrott-ing process. This carrott-ing  
solution adds considerable weight to the fur and  
may also be stored for substantial periods of  
time without deterioration. Furthermore, there  
is no discoloration of the fur and consequently  
the resultant felt may take any shades of dyes  
without undercasting or mottled effects. Fur  
carrott-ed with the above solutions will take a sub-  
stantial quantity of filler without detracting from  
its felting characteristics and is also rapid in  
starting and shrinking.

Accordingly, I have accomplished the several  
objects hereinabove mentioned as well as many  
others in a practical manner.

As the art herein described may be varied in  
various parts without departing from the scope  
of the invention, it is to be understood that all  
matter hereinbefore set forth is to be interpreted  
as illustrative and not in a limiting sense.

I claim:

1. The herein described art of preparing fur for  
felting comprising applying to the fur a solution  
of chloric acid, sulphuric acid, and potassium  
permanganate.
2. The herein described art of preparing fur  
for felting comprising applying to the fur a solution  
of chloric acid .4 molal, sulphuric acid .3  
molal, and potassium permanganate .15 molal.

WARREN C. MERCIER.